

## UNITED STATES PATENT OFFICE.

CARL AUGUST HAANEN, OF COLOGNE-MULHEIM, GERMANY, ASSIGNOR TO FELTEN & GUILLEAUME CARLSWERK ACTIEN-GESELLSCHAFT, OF COLOGNE-MULHEIM, GERMANY.

### PROCESS FOR THE PRODUCTION OF INSULATING PAPER CONTAINING PHENOL RESINS.

No Drawing. Application filed November 27, 1926, Serial No. 151,360, and in Germany April 29, 1926.

It is known to produce insulating paper, more particularly hard paper, by saturating the finished paper with solutions of phenol resins and subsequently hardening the resins.

5 The object of the present invention is a process for the production of insulating paper containing phenol resin.

The process is as follows:—

10 The water of pulps of fibrous material of any kind is first of all replaced in a suitable manner, for instance in displacing apparatus, by a solvent for phenol resins, for instance alcohol. Solutions containing phenol resins are added to the mass obtained in this 15 manner and by introducing the well mixed mass into water, the phenol resin is precipitated in and on the fibre. The resin contained in the fibre can be left as it is or converted by heat into the C-state, according to 20 the working up processes employed and the purposes in view. The resulting paper pulp is used for the manufacture of paper or hard paper as well as, after drying, for the production of pressed articles. The papers produced according to the process according to 25 the invention can be successfully used as insulation for high tension cables, the grading according to the dielectric constants, desirable therefor being obtained by the different 30 percentage content of phenol resin in the various layers of paper.

What I claim is:—

1. A process for the production of insu-

lating paper containing phenol resins, consisting in replacing the water in the fibrous pulp by solvents for phenol resins, adding 35 solutions containing phenol resins, precipitating the phenol resin in and upon the fibres by the addition of water and working up the fibrous material to form paper and 40 pressed articles.

2. A process for the production of insulating paper containing phenol resins, consisting in replacing the water in the fibrous pulp by solvents for phenol resins, adding 45 solutions containing phenol resins, precipitating the phenol resin in and upon the fibres by the addition of water, converting the resin into the C-state by the action of 50 heat and working up the fibrous material to 55 form paper and pressed articles.

3. A process for the production of insulating paper containing phenol resins, consisting in replacing the water in the fibrous pulp by solvents for phenol resins, adding 55 solutions containing phenol resins, precipitating the phenol resin in and upon the fibres by the addition of water, working up the fibrous material to form paper and 60 pressed articles and converting the resin into the C-state in the said finished paper and pressed articles.

In testimony whereof I have signed my name to this specification.

CARL AUGUST HAANEN.